

Patented May 3, 1927.

1,626,965

# UNITED STATES PATENT OFFICE.

PETER L. PAULSON, OF CLINTON, MINNESOTA.

## FIRE-KINDLING MATERIAL.

No Drawing.

Application filed September 7, 1926. Serial No. 134,130.

The present invention relates to a fire kindling material which may be made up into solid form and which will function quickly and efficiently as a kindler for coal or wood fires.

Among the objects in view are to provide an inexpensive and safe kindling material formed in convenient blocks adapted to be broken as needed, the nature of the kindler being such as to create when ignited an intense and lasting heat, which, without the aid of kindling wood, will in a very few moments thoroughly ignite the coal. The material is adapted for use in steam engine boilers, locomotive boilers, stoves, furnaces, and, in fact, anywhere wherein it is essential or desirable to provide a quick and intense heat.

With these general objects in view, the invention consists in the mixing and molding of certain ingredients, and, further in treating the same, all as will hereinafter appear and be particularly claimed.

My material is formed of the following ingredients in the proportions listed:

50 pounds resin, 25 pounds shavings (such as oak, wood, or any hard wood),  $1\frac{1}{2}$  pound rubber,  $1\frac{1}{2}$  pound coal tar creosote oil,  $1\frac{1}{2}$  pound gasoline, 1 pound celluloid.

Rubber and resin are melted together until well mixed. The celluloid is cut up into small pieces and mixed with the coal tar creosote oil and gasoline and then poured into the mixture of resin and rubber and the

resultant mixture is thoroughly stirred and 35 then poured into a suitable form and when the mixture hardens, it forms a block which may be broken off into desirable sized pieces for use in a furnace. When the resultant mixture is lighted it sets up a very intense 40 and quick heat which will ignite the coal in a few moments.

It is to be understood that the proportions mentioned above may be varied to a considerable extent but are mentioned because from my experiments they produce the 45 best results.

Having thus described my invention, what 1 claim as new is:—

1. A kindling composition of the class 50 described, including, in a mixture, resin, wood shavings, rubber, coal tar creosote oil, gasoline, and celluloid.

2. A kindling composition of the class described, composed of 50 pounds of resin, 25 pounds of wood shavings,  $1\frac{1}{2}$  pounds of rubber,  $1\frac{1}{2}$  pounds of coal tar creosote oil,  $1\frac{1}{2}$  pounds of gasoline, and one pound of celluloid.

3. The process of forming a kindling composition consisting of mixing together a quantity of rubber and resin and melting the same, then mixing together a quantity of celluloid, wood shavings, coal tar creosote oil and gasoline, and then mixing the first mixture with the second mixture.

In testimony whereof I affix my signature.

PETER L. PAULSON.